

3,208,814

**PROCESS OF COLORING TEXTILE MATERIALS WHICH COMPRISES CROSS-LINKING THE TEXTILE TO A WATER-SOLUBLE DYE-STUFF THROUGH A TRIS AZIRIDINYL PHOSPHINE COMPOUND**

Frederic L. Sievenpiper, Alden, and Leon S. Zielinski, Concord Township, Erie County, N.Y., assignors to Allied Chemical Corporation, New York, N.Y., a corporation of New York  
No Drawing. Filed June 4, 1962, Ser. No. 199,595  
9 Claims. (Cl. 8—18)

The present invention relates to a novel process for the coloration of textile materials. More particularly it relates to a process of dyeing and printing textile materials in bright shades which are characterized by their fastness to light and to washing.

It is known to color textile materials with (1) substances such as the substantive dyestuffs which are held on the fiber by relatively loose physical forces, i.e., hydrogen bonding, (2) substances which are insolubilized on the fiber such as the vat dyestuffs or azoics, (3) substances which are applied with resins or resin-forming materials and are occluded with the resin as it is formed or deposited in and on the fiber, and more recently (4) substances which react with the fiber forming a relatively strong chemical bond, i.e., the reactive dyestuffs.

Each of these classes of dyestuffs or coloring methods is deficient in one or more desirable properties which limits the utilization of the class. Thus, vat dyestuffs are generally lacking in brilliance and because they are generally applied from strongly alkaline media are limited somewhat as to the fibers to which dyestuffs can be applied. Azoic dyestuffs are not only expensive but also require multistep application procedures. Substantive dyestuffs, although less costly, are often lacking in one or more fastness properties, while reactive dyestuffs are not only expensive but exhaust poorly, and are hence wasteful. Dyestuffs occluded with resins on the fiber give rise to fabrics of inferior handle and of poor physical properties, i.e., reduced wet strength, stiffness, etc.

It is, therefore, a principal object of this invention to devise a novel process for coloring textile and related materials in bright shades of excellent fastness to light and to washing.

An ancillary object is to devise an effective method for the coloration of cellulosic fibers with non-substantive dyestuffs in shades of excellent fastness to washing.

Another object is to devise a process of coloring textile materials which is economical to operate and can be carried out in a continuous manner.

A further object is to devise a continuous dyeing process which can be operated simultaneously with one or more finishing operations.

Other objects will be obvious from the following description of our invention.

We have now devised a surprisingly effective, economical process for coloring textile and related materials to produce colorations which are remarkably fast to washing and to light. Our new process comprises impregnating the textile or related material with a solution, dispersion, emulsion, or the like of a mixture or reaction product of a water soluble dyestuff and a tris-aziridinyl phosphine oxide, hereinafter defined, such as tris-aziridinyl phosphine oxide, preferably in the presence of a catalyst, and heating the impregnated material to firmly fix the dyestuff on the fiber by cross-linking.

The dyestuffs applicable by the process of this invention are those which contain certain reactive hydrogen containing groups which provide a cross-linking site for the aziridinyl compound when activated to bind the dye-

stuffs to the textile fiber. Dyestuffs containing one or more of the same or different reactive hydrogen-containing groups can be used. Preferably the dyestuffs should possess little or no affinity for the fiber so that any coloration produced is a result of the chemical reaction, "cross-linking" rather than physical absorption or "hydrogen bonding."

Aziridinyl compounds are known in the art and have been used, either alone or in conjunction with other resin-forming compounds to impart crease-proofing, fire-proofing and the like characteristics to textile and allied materials. Such compounds have been polymerized on, or otherwise reacted with the fiber by means of catalysts (acid or alkaline) or by means of heat alone. In our experience, it has been found that the amount of monomeric aziridinyl compound which is required to provide fireproofing or crease-proofing or the like properties is far in excess of that amount which suffices to bind certain groups of water soluble dyestuffs to the fiber. Furthermore the fiber undergoes no deterioration of other properties, such as wet strength or wettability, when cross-linked to dyestuffs according to our invention.

Bis-aziridinyl compounds, such as the reaction product of hexamethylene diisocyanate and ethylene imine, when applied to the fiber in the presence or absence of dyestuffs, increase the susceptibility of the fiber to retain chlorine on bleaching the hypochlorite, which on heating, e.g., ironing, results in loss of strength of the fabric as well as of the dyeing. We have found that textile materials cross-linked to dyestuffs in accordance with the process of the present invention demonstrate a reduced susceptibility to chlorine retention on treatment with such bleaching agents.

The novel and useful improvements of the process of our invention are obtainable using an aziridinyl derivative selected from those of the following general formula,



wherein X is oxygen or sulfur and R, R<sub>1</sub>, R<sub>2</sub>, and R<sub>3</sub> are alike or different and are hydrogen or lower hydrocarbon alkyl groups.

As examples of such suitable aziridinyl compounds, the following may be mentioned:  
Tris-(1-aziridinyl) phosphine oxide  
Tris-(1-aziridinyl) phosphine sulfide  
Tris (2-methyl-1-aziridinyl) phosphine oxide  
Tris (2-methyl-3-ethyl-1-aziridinyl) phosphine oxide  
Tris (2-amyl-1-aziridinyl) phosphine oxide

Although these aziridinyl compounds can be activated, that is, caused to crosslink the dyestuff with the fiber by means of heat alone or in the presence of an acid or basic catalyst, we prefer to use heat and an acid liberating catalyst.

As examples of suitable catalysts, the following may be given:

Zinc fluoborate  
Zinc chloride  
Zinc nitrite  
Ammonium rhodanide  
Ammonium chloride  
Trimethyl amine hydrochloride  
Tris (2-hydroxyethyl) amine hydrochloride  
2-amino-2-methyl-1-propanol hydrochloride

The dyestuffs operative in our novel process are those water soluble dyestuffs, preferably acid wool dyestuffs, which contain at least one reactive hydrogen, that is a

hydrogen capable of reacting with an activated aziridinyl compound and thus to effect one portion of the cross-linking operation. However, it has been found that not all such dyestuffs are satisfactory, and for purposes of our invention those dyestuffs having hydrogen containing radicals of the group consisting of amino, imino, carbonamido



sulfonamido ( $-\text{SO}_2\text{NH}-$ ), and alcoholic and phenolic hydroxyl are suitable.

Water soluble metallized dyestuffs generally can be crosslinked particularly well with the textile material according to our novel process, and hence constitute a preferred class of dyestuffs therefor. Such dyestuffs, as is well known, are obtained by heating a dyestuff containing chelatable groups, e.g., O,O'-dihydroxyazo-, O-hydroxy-O'-carboxyazo-, O-hydroxy carboxy, etc. groups, with a Werner complex forming metal, e.g., chromium, cobalt, copper, nickel, etc. Such metallized water-soluble dyes preferably contain reactive groups in addition to the hydroxy group present in the chelatable moiety.

The amount of tris-aziridinyl compounds of the type described above which can be used to effect cross-linking of the dyestuff and the textile material can be varied over a broad range. The minimum amount is that which is necessary to react with the dyestuff present and to effect a cross-linking attachment to the fiber. This reaction, we believe, involves a separate aziridinyl moiety for each linkage as indicated by the following reactions which may occur in any order:



The remaining aziridinyl group can react with another molecule of dyestuff or with another cellulosic hydroxyl group. According to this hypothetical cross-linking mechanism of our process, it can be seen that 1 mole of tris-aziridinyl compound is equivalent to one or a maximum of two moles of a dyestuff which contains one reactive hydrogen.

The invention is preferably and most economically carried out by applying an aqueous liquor containing the tris-aziridinyl compound and dyestuff reactive therewith to the textile goods and then heating to effect a cross-linking reaction chemically bonding the dyestuff and fiber, as discussed above. However, the invention is not limited thereto but includes in its broad scope a process wherein the tris-aziridinyl compound and dyestuff reactive therewith are first reacted in the absence of the textile to produce a dyestuff containing at least one aziridinyl group, e.g.,



The dyestuff thus obtained is then applied to the textile and heated (preferably in the presence of an acidic catalyst) to cause one or both of the unreacted aziridinyl

groups to react with the textile, e.g., cotton, and thereby chemically bond the dyestuff to the textile. In any event, it is necessary to apply the dyestuff and tris-aziridinyl compound to the textile simultaneously. It has been found that stepwise addition of the dyestuff and cross-linking agent results in a considerably inferior fixation of the dyestuff to the textile. It is also interesting to note that omission of the heating step, during which most, if not all, of the cross-linking occurs, results in a colored fabric from which the color can be removed substantially completely by the same soaping or scouring treatment described in the examples.

We prefer to use an excess over such theoretical proportion of the tris-aziridinyl compound, and hence our preferred amount is from 2 to about 6 moles of tris-aziridinyl compound per mole of dyestuff containing a suitable reactive hydrogen group. The use of more than about 6 moles of tris-aziridinyl compound per mole of dyestuff is generally not required for the cross-linking operation and such excess amounts, while desirable in instances where the coloration process is to be combined with a crease proofing and/or fireproofing step, are not harmful to the basic process.

The excellent light fastness properties characteristic of 25 dyes obtained by our novel process are surprising since it is well known that such properties are often substantially affected by chemical modification of the dyestuff molecule as well as by resin finishings applied to textiles.

This new process is applicable to textile materials 30 derived from natural or synthetic fibers which contain a group or groups reactive with aziridinyl compounds. Thus the novel process is effective not only for cotton but also for other cellulosic materials, such as cellulose acetate and regenerated cellulose, polyacrylonitrile, polyesters, 35 polyamides, silk, wool and various blends and mixtures of such natural and synthetic fibers.

The new process is adaptable to the coloration (i.e., dyeing and/or printing) of not only textile and related materials, e.g., woven fabrics, yarns, fibers (felted or 40 unfelted), films, foils and the like. It can be used to color paper, also.

Our novel process is especially adaptable to continuous processes for coloring of textile materials, e.g., the "pad-steam" or "pad-dry and cure" processes, wherein high 45 speeds and short contact times are generally used. Our preferred procedure, in which an acid (or acid liberating) catalyst is used, accomplishes the cross-linking in about 3 to 5 minutes, which is generally adequate for such continuous dyeing operation.

When acid catalysts are not used to promote the cross-linking operation during the heating step, 10 to 30 minutes or more may be required to complete the reaction.

The following examples illustrate the invention. Parts and percentages are by weight and temperatures are 55 given in degrees centigrade.

#### EXAMPLE 1

A solution containing 2 parts (approximately 0.0027 mole) of Solantine Turquoise FBL (copper phthalocyanine containing one ammonium sulfonate and one sulfonamido group), 1 part (0.00578 mole) of tris(1-aziridinyl) phosphine oxide (as an 85% by weight solution in ethanol), 192 parts of water, 1 part of dispersing agent (Triton X-100, an alkyl aryl polyether alcohol, Rohm and Haas Co.), 2 parts of triethylamine and 2 parts of 60 40% aqueous zinc fluoroborate was padded on cotton broadcloth (20 parts). The material was passed through squeeze rollers to express excess padding liquor, after which the material retained about 80% of its weight of 65 padding solution (percent pickup). The fabric was dried for 5 minutes at 75° to 80° under slight tension in a stream of air. A portion of the impregnated fabric was baked at 155° ± 5° for ten minutes and then rinsed in 1000 parts of water at ambient temperature for 1 to 2 minutes. The baked fabric portion was rinsed in hot 70 75

water (80°), scoured by boiling for ten minutes in 1000 parts of an aqueous 0.2% solution of Triton X-100 and dried at 75° to 80° in a stream of air.

The amount of dyestuff cross-linked to the cotton fabric in this manner was estimated by comparison of the baked and unbaked fabric portions and by the visual determination of the amount of color bleed in the cold water rinsing and scouring steps. This is estimated by diluting an aliquot of the original padding liquor (the dye strength of which is known) until the intensity of color of the diluted aliquot is equal to the intensity of color in the combined rinse and scour liquors. From the amount of dyestuff padded onto the cloth and the amount of dyestuff in the rinse and scour liquors, the amount of dyestuff cross-linked to the fabric can be estimated.

In this example, about 70% of the dyestuff was cross-

linked to the cotton fabric, which was colored a bright greenish blue shade having excellent fastness to washing.

#### EXAMPLES 2 TO 9

5 The procedure of Example 1 was repeated in a number of experiments wherein the quantities of cross-linking agent, water and/or dye employed in the padding solution were varied. The results of these experiments are shown in Table I.

10

#### EXAMPLES 10 TO 69

The procedure described in Example 1 was carried out with various dyestuffs while varying the components of the padding solution. The results of these experiments are shown in Table II.

15

"Fixation" in Examples 2-70 was determined by the comparison technique described in Example 1.

Table I

[All quantities are in parts by weight unless otherwise noted]

| Example                 | 2                | 3                | 4                 | 5                 | 6                 | 7                 | 8                  | 9                    |
|-------------------------|------------------|------------------|-------------------|-------------------|-------------------|-------------------|--------------------|----------------------|
| Solantine Turquoise FBL | 2 (0.0027 mole). | 2 (0.0027 mole). | 2 (0.0027 mole).  | 2 (0.0027 mole).  | 2 (0.0027 mole).  | 1 (0.00133 mole). | 0.75 (0.001 mole). | 0.5 (0.000665 mole). |
| Water                   | 193              | 191              | 190               | 187               | 184               | 188               | 188                | 188.5                |
| APQ                     | 0                | 2 (0.0116 mole). | 3 (0.0173 mole).  | 6 (0.0347 mole).  | 9 (0.0518 mole).  | 6 (0.0347 mole).  | 6 (0.0347 mole).   | 6 (0.0347 mole).     |
| Dye Fixation            | Very poor (0%).  | Good (70%).      | Excellent (100%). | Excellent (100%). | Excellent (100%). | Excellent (100%). | Excellent (100%).  | Excellent (100%).    |

\*Tris-(1-aziridinyl) phosphine oxide (85% by weight in ethanol).

Table II

| Example | Notes               | Dyestuff                                                                                               | Parts | Parts <sup>4</sup> Cross-Linking Agent | Parts <sup>5</sup> Catalyst | Parts <sup>6</sup> Buffer | Parts <sup>7</sup> Dispersing Agent | Parts Water | Fixation           |
|---------|---------------------|--------------------------------------------------------------------------------------------------------|-------|----------------------------------------|-----------------------------|---------------------------|-------------------------------------|-------------|--------------------|
| 10.     | ( <sup>1</sup> 3)   | Benzidine 2,2'-disulfo acid → salicylic acid                                                           | 4     | 6                                      | 1                           | None                      | 1                                   | 188         | Excellent.         |
| 11.     | ( <sup>1</sup> 2)   | 1,6-diamino-4,8-dihydroxy anthraquinone-3-sodium sulfonate.                                            | 4     | 6                                      | 1                           | None                      | 1                                   | 188         | Good to excellent. |
| 12.     | ( <sup>1</sup> 3)   | H acid → 1 (p-tolyl) amino naphthyl-8-sodium sulfonate.                                                | 4     | 6                                      | 1                           | None                      | 1                                   | 188         | Excellent.         |
| 13.     | ( <sup>1</sup> 3)   | P-Aminosulfo salicylic acid → 1,6 Cleves → N (p-salicyl sulfo) H acid.                                 | 4     | 6                                      | 2                           | None                      | 1                                   | 187         | Very good.         |
| 14.     | ( <sup>1</sup> 2 2) | 2-aminonaphthyl 4,8-disodium sulfonate → m-toluidine.                                                  | 10    | 6                                      | 2                           | 1.5                       | 1                                   | 180         | Excellent.         |
| 15.     | ( <sup>1</sup> )    | Benzidine 2,2'-disulfo acid → N (p-salicyl sulfo) H acid.                                              | 4     | 6                                      | 2                           | None                      | 1                                   | 187         | Do.                |
| 16.     | ( <sup>1</sup> )    | 3-amino-4-hydroxybenzene sulfonamide → 1-naphthol-5-sodium sulfonate chrome complex (2:1).             | 2     | 12                                     | 2                           | None                      | 1                                   | 183         | Do.                |
| 17.     | ( <sup>1</sup> )    | Benzidine 2,2'-disulfonic acid → R salt.                                                               | 2     | 12                                     | 2                           | None                      | 1                                   | 183         | Good to excellent. |
| 18.     | ( <sup>1</sup> )    | Chromium (2:1) complex of 3-amino-4-hydroxy benzene sulfonamide → H acid.                              | 4     | 6                                      | 2                           | None                      | 1                                   | 187         | Excellent.         |
| 19.     | ( <sup>1</sup> )    | Nitro-1,2,4-acid → H acid (chromed 2:1).                                                               | 4     | 6                                      | 2                           | None                      | 1                                   | 187         | Do.                |
| 20.     | ( <sup>1</sup> )    | Mixture of 2:4 parts dye of Ex. 19 + 1.6 parts of dye of Ex. 16.                                       | 1.6   | 10                                     | 2                           | None                      | 1                                   | 133         | Do.                |
| 21.     | ( <sup>1</sup> )    | Chromium complex of 6-amino 1,2,4 acid → H acid (chromed).                                             | 4     | 10                                     | 2                           | None                      | 1                                   | 183         | Do.                |
| 22.     | ( <sup>1</sup> )    | 3-amino-4-hydroxybenzene sulfonamide → (m-amino-phenyl) 3-carboxy-5-pyrazolone (chromed).              | 4     | 10                                     | 2                           | None                      | 1                                   | 183         | Do.                |
| 23.     | ( <sup>1</sup> )    | Cobalt complex of dye of Ex. 22.                                                                       | 6     | 9                                      | 3                           | 1.5                       | 1.5                                 | 279         | Do.                |
| 24.     | ( <sup>1</sup> )    | 2-naphthylamino-4,8-disulfonic acid → N-(3,5-bis (2-aminoethyl-amino) triazinyl-1) m-toluidine.        | 3     | 6                                      | 2                           | 2                         | 1                                   | 186         | Very good.         |
| 25.     | ( <sup>1</sup> )    | Copper phthalocyanine containing 2-sulfonic acid and 2-sulfonamide groups.                             | 3     | 6                                      | 2                           | 1                         | 1                                   | 187         | Excellent.         |
| 26.     | ( <sup>1</sup> )    | 6-(5-amino-2H-benzotriazolyl) 1,2,4-acid → H acid.                                                     | 4     | 6                                      | 2                           | 1                         | 1                                   | 187         | Do.                |
| 26a.    | ( <sup>1</sup> )    | 1-amino-2-hydroxy-naphthalene-4-sulfo acid → 1 (m-sulfonylphenyl) 3-methyl-5-pyrazolone (chromed).     | 4     | 6                                      | 2                           | ( <sup>8</sup> )          | 1                                   | 187         | Do.                |
| 27.     |                     | Chromium complex of 3-amino-4-hydroxybenzene sulfonic acid → 1 (m-aminophenyl) 3-carboxy-5-pyrazolone. | 4     | 10                                     | 3                           | 2                         | 1                                   | 180         | Do.                |
| 28.     |                     | Chromium complex of mono-sulfonic acid of anthranilic acid → 1 (m-aminophenyl) 3-carboxy-5-pyrazolone. | 2     | 6                                      | 2                           | 1                         | 1                                   | 189         | Do.                |
| 29.     |                     | Copper complex of dye of Ex. 28.                                                                       | 2     | 6                                      | 2                           | 1                         | 1                                   | 189         | Do.                |
| 30.     |                     | Chromium complex of nitro-1,2,4 acid → S acid.                                                         | 2     | 6                                      | 2                           | 1                         | 1                                   | 189         | Do.                |
| 31.     |                     | Cobalt complex of dye of Ex. 30.                                                                       | 2     | 6                                      | 2                           | 1                         | 1                                   | 189         | Do.                |
| 32.     |                     | Chrome complex of nitro-1,2,4 acid → SS acid.                                                          | 2     | 6                                      | 2                           | 1                         | 1                                   | 189         | Do.                |
| 33.     |                     | Chromium complex of 3-amino-4-hydroxy-5-nitrobenzene-sulfonic acid → SS acid.                          | 2     | 6                                      | 2                           | 1                         | 1                                   | 189         | Do.                |
| 34.     |                     | Cobalt complex of dye of Ex. 32.                                                                       | 2     | 6                                      | 2                           | 1                         | 1                                   | 189         | Do.                |
| 35.     |                     | Chromium complex of 3-amino-4-hydroxy-5-nitrobenzene sulfic acid → S acid.                             | 2     | 6                                      | 2                           | 1                         | 1                                   | 189         | Do.                |
| 36.     |                     | Cobalt complex of dye of Ex. 35.                                                                       | 2     | 6                                      | 2                           | 1                         | 1                                   | 189         | Do.                |
| 37.     |                     | Chromium complex of dye of Ex. 35. Nitro group reduced to amino.                                       | 2     | 6                                      | 2                           | 1                         | 1                                   | 189         | Do.                |
| 38.     |                     | Cobalt complex of dye of Ex. 28.                                                                       | 2     | 6                                      | 2                           | 1                         | 1                                   | 189         | Do.                |
| 39.     |                     | N-(2-aminoethyl)sulfamyl copper phthalocyanine monosulfonic acid.                                      | 10    | 12                                     | 4                           | 2                         | 2                                   | 371         | Do.                |

See footnotes at end of table.

Table II—Continued

| Example | Notes | Dyestuff                                                                                                                           | Parts | Parts <sup>6</sup> Cross-Linking Agent | Parts <sup>8</sup> Catalyst | Parts <sup>8</sup> Buffer | Parts <sup>7</sup> Dispersing Agent | Parts Water | Fixation           |
|---------|-------|------------------------------------------------------------------------------------------------------------------------------------|-------|----------------------------------------|-----------------------------|---------------------------|-------------------------------------|-------------|--------------------|
| 40      |       | 3-amino-4-hydroxy-2-nitrobenzene sulfo acid →1(2-chloro-5-sulfonyl)3-methyl-5-pyrazolone; reduced →2,4-diamino benzene sulfo acid. | 2     | 6                                      | 2                           | 1                         | 1                                   | 188         | Do.                |
| 41      |       | 6(5-amino-6-sulfo-2H-benzotriazolyl)-1,2,4-acid →1(2-chloro-5-sulfonyl)3-methyl-5-pyrazolone.                                      | 2     | 6                                      | 2                           | 1                         | 1                                   | 188         | Do.                |
| 42      |       | Chromium complex of 6-amino-1,2,4-acid →1(2-chloro-5-sulfonyl)3-methyl-5-pyrazolone.                                               | 2     | 6                                      | 2                           | 1                         | 1                                   | 188         | Do.                |
| 43      |       | Cobalt complex of dye of Ex. 42                                                                                                    | 2     | 6                                      | 2                           | 1                         | 1                                   | 188         | Do.                |
| 44      |       | Dehydrothio p-toluidinesulfonic acid →aceto-acetylaminobenzene-4-sulfo acid.                                                       | 4     | 10                                     | 3                           | 2                         | 2                                   | 170         | Do.                |
| 45      |       | N(3-sulfamylphenyl)-3-nitrosulfanilic acid                                                                                         | 4     | 10                                     | 3                           | 1                         | 1                                   | 181         | Good to excellent. |
| 46      |       | Same as Ex. 45                                                                                                                     | 4     | 10                                     | 10 <sup>4</sup>             | 1                         | 1                                   | 180         | Do.                |
| 47      |       | Chromium complex of 6(5-amino-2H-benzotriazolyl)-1,2,4-acid →H acid.                                                               | 6     | 12                                     | 3                           | 2                         | 2                                   | 175         | Excellent.         |
| 48      |       | Cobalt complex of 6-nitro-1,2,4-acid →SS acid.                                                                                     | 1     | 6                                      | 2                           | 1                         | 2                                   | 188         | Do.                |
| 49      |       | Chrome complex of 3-amino-4-hydroxy-5-nitrobenzene sulfonic acid →S acid, reduced.                                                 | 4     | 6                                      | 2                           | 2                         | 2                                   | 184         | Do.                |
| 50      |       | Cobalt complex of dye of Ex. 49                                                                                                    | 4     | 6                                      | 2                           | 2                         | 2                                   | 184         | Do.                |
| 51      |       | 1-amino-4(4'-aminophenylamino)anthraquinone 2,3'-disulfonic acid.                                                                  | 2     | 6                                      | 2                           | 1                         | 2                                   | 187         | Do.                |
| 52      |       | Cobalt complex of 3-amino-4-hydroxy-5-nitrobenzene sulfonic acid →S acid.                                                          | 1     | 6                                      | 2                           | 1                         | 2                                   | 187         | Do.                |
| 53      |       | Cobalt complex of 3-amino-4-hydroxy-5-nitrobenzene sulfonic acid →SS acid.                                                         | 1     | 6                                      | 2                           | 1                         | 2                                   | 187         | Do.                |
| 54      |       | Chromium complex of 3-amino-4-hydroxybenzene sulfonic acid →H acid.                                                                | 1     | 6                                      | 2                           | 1                         | 2                                   | 187         | Do.                |
| 55      |       | 1,8-diamino-4,5-dihydroxy anthraquinone-3,6-disulfo acid.                                                                          | 2     | 10                                     | 3                           | 1                         | 1                                   | 188         | Very good.         |
| 56      |       | Naphthionic acid →benzidine →phenol (treated with benzene sulfonyl chloride).                                                      | 4     | 6                                      | 2                           | 2                         | 1                                   | 185         | Do.                |
| 57      |       | Gamma acid →p-phenylene diamine →phenol (treated with benzene sulfonyl chloride).                                                  | 4     | 6                                      | 2                           | 2                         | 1                                   | 185         | Do.                |
| 58      |       | 4,4'-isopropylidene dianiline →1(2-chloro-5-sulfonyl)-3-methyl-5-pyrazolone.                                                       | 4     | 6                                      | 2                           | 2                         | 1                                   | 185         | Do.                |
| 59      |       | Chromium complex (2:1) of dye of Ex. 26                                                                                            | 4     | 6                                      | 2                           | 2                         | 1                                   | 185         | Excellent.         |
| 60      |       | Chromium complex (2:1) of 3-amino-2-hydroxybenzene 1,5-disulfo acid →1(3'-aminophenyl) 3-carboxy-5-pyrazolone.                     | 4     | 6                                      | 2                           | 2                         | 1                                   | 185         | Very good.         |
| 61      |       | Chromium complex (2:1) of 3-amino-2-hydroxy-5-nitrobenzene sulfonic acid →1(3'-aminophenyl) 3-carboxy-5-pyrazolone.                | 4     | 6                                      | 2                           | 2                         | 1                                   | 185         | Do.                |
| 62      |       | Chromium complex (2:1) of 2-amino-4-sulfobenzoic acid →1(p-aminophenyl)3-methyl-5-pyrazolone.                                      | 2     | 12                                     | 3                           | 2                         | 1                                   | 180         | Do.                |
| 63      |       | 3-amino-4-chlorobenzene sulfonic acid →1(p-aminophenyl)3-methyl-5-pyrazolone.                                                      | 2     | 12                                     | 3                           | 1                         | 1                                   | 181         | Excellent.         |
| 64      |       | 2-aminonaphthalene-6-sulfo acid →1-hydroxy-6(m-amino-benzoyl)aminonaphthalene 3-sulfonic acid.                                     | 2     | 10                                     | 3                           | 2                         | 1                                   | 182         | Very good.         |
| 65      |       | 2-amino-6-chloro-3-methyl benzene sulfonic acid →1(m-aminophenyl)3-carboxy-5-pyrazolone.                                           | 4     | 20                                     | 6                           | 2                         | 1                                   | 167         | Do.                |
| 66      |       | Cobalt complex of 3-amino-4-hydroxybenzene sulfonamide →2-hydroxynaphthalene 3,6-disulfo acid.                                     | 4     | 6                                      | 2                           | 2                         | 1                                   | 185         | Do.                |
| 67      |       | Nickel complex of 3-amino-5-chloro-2-hydroxybenzene sulfonic acid →(m-amino-phenyl) 3-carboxy-5-pyrazolone.                        | 4     | 6                                      | 2                           | 2                         | 1                                   | 185         | Do.                |
| 68      | (*)   | Dyestuff of Ex. 23                                                                                                                 | 4     | 6                                      | 2                           | 1                         | 1                                   | 166         | Excellent.         |
| 69      |       | Dyestuff of Ex. 23                                                                                                                 | 4     | (11)                                   | 6                           | None                      | 1                                   | 183         | Do.                |

<sup>1</sup> Fabric dyed was cotton twill (20 parts).<sup>2</sup> Scouring solution was 1,000 parts 0.25% aqueous Ivory Snow.<sup>3</sup> After scouring the fabric was treated with 0.1 N aqueous hydrochloric acid (pH=3) for 30 minutes at 60° and rescored.<sup>4</sup> To the padding solution, 20 parts of 10% aqueous Methocel (methyl cellulose, Dow Chemical Co.) were added to afford a more level dyeing.<sup>5</sup> Parts 40% aqueous Zn fluoroborate unless otherwise noted.<sup>6</sup> Tris (1-aziridinyl) phosphine oxide (85% solution in ethyl alcohol) unless otherwise noted.<sup>7</sup> Triton X-100 unless otherwise noted.<sup>8</sup> Triethylamine unless otherwise noted.<sup>9</sup> Triethanol amine.<sup>10</sup> 2-amino-2-methyl-1-propanol hydrochloride (Catalyst AC).<sup>11</sup> Tris (1-aziridinyl) phosphine sulfide.

fixation of dye in both experiments was rated as excellent, i.e., substantially complete cross-linking of the dyestuff.

## EXAMPLE 71

(A) A padding liquor was prepared consisting of:

|                                       | Parts | Percent |
|---------------------------------------|-------|---------|
| Red Dyestuff *                        | 15    | 1.5     |
| Water                                 | 546   | 92.0    |
| Triton X-100                          | 3     | 0.5     |
| Tris aziridinyl phosphine oxide (85%) | 27    | 4.5     |
| Zinc Fluoroborate (40% solution)      | 9     | 1.5     |

\* Dyestuff used was the chromium complex of the dyestuff from diazotized 2-aminophenol-4-sulfonic acid coupled into 1(m-aminophenyl)-3-carboxy-5-pyrazolone; it contained 60% coal tar dye solids or 15 parts of the dye composition contained 9 parts of 100% dyestuff, the balance, 6 parts, being essentially inorganic salts.

A 6" x 15" strip of polycaproamide cloth was padded therewith in a conventional three roll padder operating at a pressure of 200 lbs. on the rolls. The pickup was

The following example illustrates the application of the present process to textile printing. A mixture of 1 part of the dyestuff of Example 1, 2 parts of Pluronic F-68 (a high molecular weight nonionic surfactant prepared by condensing ethylene oxide with a hydrophobic base formed by the condensation of propylene oxide with propylene glycol; Wyandotte Chemical Corp.) and 43 parts of water was adjusted to a pH of 9 by the addition of sodium carbonate and 50 parts of 4% aqueous Methocel (methyl cellulose, Dow Chemical Co.), 3 parts of tris (1-aziridinyl) phosphine oxide (as an 85% solution in ethyl alcohol), 1 part 40% aqueous zinc fluoroborate were added. The mixture was printed on cotton broadcloth and dried, baked and subsequently treated substantially as described in Example 1. In another experiment, the foregoing procedure was repeated except that impregnated material was baked without being dried. The



11

the dyestuff molecule attaches to the carbon of the cleaved ring.

## References Cited by the Examiner

## UNITED STATES PATENTS

3,044,843 7/62 Tullio ----- 8-17  
3,084,017 4/63 Reeves et al. ----- 8-18

12

## OTHER REFERENCES

Broden et al.: Amer. Dyestuff Reporter, Jan. 4, 1954,  
pp. P6-P13.

5 NORMAN G. TORCHIN, Primary Examiner.  
ABRAHAM H. WINKELSTEIN, Examiner.